

# UNITED STATES PATENT OFFICE.

ARTHUR GRANVILLE, OF LONDON, ENGLAND, ASSIGNOR TO THE FUR-WOOL COMPANY LIMITED, OF LONDON, ENGLAND, A CORPORATION.

## PROCESS OF TREATING SKINS.

No. 866,458.

Specification of Letters Patent.

Patented Sept. 17, 1907.

Application filed July 25, 1906. Serial No. 327,780.

*To all whom it may concern:*

Be it known that I, ARTHUR GRANVILLE, a subject of the King of Great Britain, residing at London, England, have invented certain new and useful Improvements in the Processes of Treating Skins; and I do hereby declare the following to be a full, clear, and exact description of the invention, such as will enable others skilled in the art to which it appertains to make and use the same.

10 My invention relates to the obtainment of a new kind of fur from lamb and such like skins, as hereafter described. I have discovered that such skins have two layers of wool upon them the second layer lying close to the skin; and is covered by the other layer so that it is not seen. This under layer is of much finer character than the outer layer and has a tendency to curl close to the skin. The way in which skins are now dressed spoils this natural tendency to curl and frequently destroys the curl altogether, causing the wool to draw out 15 straight similar to the outside layer so that the two mix and in the cutting off of the outside layer a portion of the under layer is cut away and but little curl is left upon the skin. The way I have discovered for dressing skins does not spoil the curl of the under wool, and 20 25 by special attention to the cutting I can take-off only the outside layer of wool leaving the curly wool upon the skin. By this means I obtain a novel fur of high commercial value.

My process for dressing skins is as follows.—I take 30 suitable raw skins as imported or otherwise obtained, and soak them in cold water for about ten hours and after allowing them to drain, rinse them in clean cold water. I then immerse them in dilute hydrochloric acid, say five per cent of acid to water by weight, and agitate 35 them in this solution for from two to three hours the more they are agitated in the solution the less time this operation need last; the skins are then removed and left to drain and continually well shaken during the draining, they are then to be well rinsed in cold water 40 slightly alkaline, say by having dissolved in it about

three per cent by weight to the water of borax, or about two per cent of potash, the borax being preferred. The skins are then removed from this solution and well shaken and afterwards scoured cold to cleanse the wool, after which they are tanned, and dyed in the 45 usual way. After being well dried the skins are ready for the cutting off of the outer layer of wool according to this invention.

In carrying out the operation of cutting off the outer layer of wool shearing combs are used. Several of 50 these combs are necessary to be available with different thicknesses of comb, the thickness of the comb being for keeping the cutting edge above the curl. The proper thickness of comb to be used for different skins, will only be ascertained by the examination of the wool 55 of each skin by the operator, as in some skins the curly part is thicker than in other skins. Skins which have not been dressed in the above manner can have the outer layer of wool cut off as described but the fur so obtained has not so good an appearance as when the skin 60 is first dressed as described.

Other means than shearing combs may be used to cut off the outside layer of wool, such for example, as the shaving means used in the manufacture of velvet.

Having now described my invention, what I desire 65 to secure by Letters Patent of the United States is.—

1. The process of treating skins, which consists in soaking them, treating them with a dilute acid solution, and then a dilute alkaline solution, scouring and tanning them, and finally cutting off the outer layer of wool, substantially as described. 70

2. The process of treating skins, which consists in soaking them in water, treating them with an acid solution, treating them with an alkaline solution, scouring them, tanning and drying them, and finally cutting off the outer layer of wool, the whole treatment being conducted 75 in the cold.

In testimony whereof, I have affixed my signature, in presence of two witnesses.

ARTHUR GRANVILLE.

Witnesses:

FREDERIC PRINCE,  
H. D. JAMESON.